

May 5, 1936.

E. W. ADAMS ET AL

2,039,377

HARD WATER SOLUBLE OIL

Filed May 20, 1933



Inventors:

Elmer W. Adams  
George W. Flint

BY *Donald E. Payne*

ATTORNEY

## UNITED STATES PATENT OFFICE

2,039,377

## HARD WATER SOLUBLE OIL

Elmer Wade Adams, Hammond, Ind., and George W. Flint, Chicago, Ill., assignors to Standard Oil Company, Chicago, Ill., a corporation of Indiana

Application May 20, 1933, Serial No. 672,050

3 Claims.

(Cl. 87—9)

This invention relates to soluble oils and it pertains more particularly to a method and means of emulsifying petroleum oils in hard water.

Soluble oils are oils containing dissolved emulsifying agents so that when they are poured into water they immediately form stable emulsions without necessity of special dispersing means, which are suitable for use as cutting oils, drawing oils, textile or wool oils, tree sprays, lubricants, coal sprays, antirust oils or any other use for which soluble oils are usually employed.

A large variety of substances have been used in the manufacture of soluble oils, particularly fatty acid soaps, naphthenic soaps, sulfonic soaps, oleic acid, sulfonated compounds, etc. In most of these soluble oils it has been necessary to use a small amount of alcohol for obtaining the desired surface tension characteristics, for stabilizing the soluble oil against low temperatures and for improving the dispersion of the soluble oil on admixture with water. The use of alcohol is objectionable not only because of its expense, but because it tends to evaporate from the finished product and it thereby causes deterioration prior to use. An object of our invention is to provide a soluble oil which does not require the use of alcohol.

Most soluble oils are quite satisfactory with ordinary soft waters but they cannot be satisfactorily used in hard waters because the calcium and magnesium compounds upset the delicate balance between interfacial tensions which is necessary for satisfactory emulsification. An object of our invention is to provide a soluble oil which will produce excellent emulsions in extremely hard water which will not cream and separate oil on standing, as a result of insufficiently small particle size.

A further object of our invention is to provide a highly efficient soluble oil employing mahogany soap, soda rosin soap or its equivalent, and an amount of water which is just sufficient to produce an excellent emulsion but is insufficient to cause the separation of soaps from the oil, during storage, in transit or prior to actual use. Other objects of the invention will be apparent from the following detailed description.

It has long been known that mahogany soap (preferentially oil soluble mineral oil sulfonates) has the property, when dissolved in oil, of lowering the surface tension of the oil and thereby promoting the emulsification of the oil in water (see Petrow 1,230,599). It has always been necessary to supplement this mahogany soap with a water-soluble soap and with small amounts of alcohol. We have discovered that by careful purifying or fractionating the mahogany soap, and by carefully regulating the proportions of this improved material with soda rosin soap or its equivalent we may eliminate the use of alcohol entirely and at the

same time obtain the soluble oil which is extremely stable at very low temperatures, which is non-corrosive and which, when poured in water, gives an emulsion which does not readily separate out even with the hardest waters.

The preferred formula for our improved soluble oil is about as follows:

|                                    | Per cent |
|------------------------------------|----------|
| Mahogany soap (purified, oil-free) | 12       |
| Soda rosin soap                    | 2.5 10   |
| Water                              | 1.5      |
| Oil                                | 84.0     |

The mahogany soap may in general be prepared as described in the United States patent 1,286,179, in the manufacture of white oils, medicinal oils and the like. Mineral oils are treated with a number of dumps of concentrated or fuming sulfuric acid, and the resulting sludge is separated from the oil after each dump. The so-called green acids are separated with the sludge and withdrawn, and the preferentially oil-soluble sulfonic acids remain dissolved in the oil. These acids are neutralized to form soaps and the soaps are extracted with 50% aqueous alcoholic solutions. These so-called mahogany soaps contain considerable amounts of oil. They also contain considerable amounts of sodium sulfate which is either dispersed or dissolved, or may be in chemical combination with the mahogany soap, since it remains in the oil phase when the green acid soap and sludge are separated. The sodium sulfate may be removed from the mahogany soap by further extraction with concentrated alcoholic solutions, as disclosed in United States Patents 1,493,111 and 1,708,838. When the mahogany soap is extracted with 80% alcohol, we find that this concentrated alcoholic solution not only removes impurities such as sodium sulfate, but that it tends to further fractionate the mahogany soap itself, and we have found that the purified mahogany soap remaining dissolved has new and unexpected properties when employed in soluble oils in the manner described.

The soda rosin soap may be prepared in the conventional manner and it may be replaced in our formula by any other equivalent water-soluble soap. We prefer to use a relatively light mineral oil, for instance, one having a viscosity between 80 and 300 seconds at 100° F. The oil may have received any degree of refinement by conventional acid treatments, solvent extraction treatments, claying treatments, etc., the type of oil used depending primarily upon the use for which it is designed.

The process of manufacture is as follows: The mahogany soap is first purified by mixing one part of soap with one and one-half parts of 78-80% (by volume) alcohol. The two are thoroughly mixed at 140-150° F. and then cooled to 60

80° F. or lower. After settling, the solution of light colored soap is separated, the final product being freed from alcohol and designated as purified mahogany soap.

The purified mahogany soap and soda rosin soap are heated and agitated in a mixer in the proportions hereinabove set forth. The heating is continued to drive off water so that the total water content will be less than 1½%, based on the finished product. The mineral oil is then added with continued stirring or blowing, the mahogany soap, soda rosin soap and water dissolving therein. Soluble oils made in this manner may be cooled to extremely low temperatures and may be stored in an ice-box for days without separating out or becoming cloudy. When this oil is added to water, even if the water is extremely hard, it immediately emulsifies without the separation of any oil at the surface.

An important part of the invention is the elimination of sodium sulfate and other undesirable salts from soluble oils of this general type. We have found that the emulsibility of an oil is materially lowered by the presence of salts. A series of oils were made by adding various amounts of a salt ( $Na_2SO_4$ ) solution of known concentration to the oil, drying the oils and bringing them back to approximately the same water content. The effect of the salt on emulsibility is shown by the following table:

| Percent original salt | cc. salt solution added | Percent salt in oil | Equivalent salt in soap stock | Emulsibility      |                    |
|-----------------------|-------------------------|---------------------|-------------------------------|-------------------|--------------------|
|                       |                         |                     |                               | In cold tap water | In cold hard water |
| 35                    | 0.24                    | 0                   | 0.24                          | 1.00              | Excellent          |
|                       | 0.24                    | 1                   | 0.40                          | 1.66              | Excellent          |
|                       | 0.24                    | 2                   | 0.56                          | 2.33              | Good               |
|                       | 0.24                    | 3                   | 0.72                          | 3.00              | No good            |
| 40                    | 0.24                    | 4                   | 0.88                          | 3.66              | No good            |
|                       | 0.24                    | 5                   | 1.04                          | 4.33              | No good            |

We have found that the salt content in our mahogany soap stock (50% soap) must be maintained as near to one percent or below as is possible, determined by the following method: The ether solution of mahogany soap and oil is washed with hydrochloric acid and diluted with three parts of water to break down the soap. This mineral acid solution is saved, dried and weighed. From this weight the sodium chloride formed from the decomposition of the soap and calculated from the titration of the acid is deducted.

Even when the highly purified or fractionated mahogany soap is used as the basic emulsifying agent it is still necessary to carefully regulate the proportions of water-soluble soap and water if the resulting soluble oil is to pass all specifications without the use of alcohol. The purified mahogany soap content may vary over relatively wide ranges, but it should not go below about 8%, and for practical purposes it will not be above 40%. An increase in the mahogany soap content permits a decrease in the mahogany-rosin soap ratio and/or an increase in the water content. In general, an increase in oil viscosity requires a slight increase in total emulsifying agent.

With a mahogany soap content of 12% the soda rosin soap content may vary from about 1% to 6% and the water content from about 2.5% to 0.5%. If 8% of soda rosin soap is used with 12% of mahogany soap the emulsifying agent separates out from the oil at low temperatures. The soluble oil should show no separation of water and emulsifying agent after long standing,—at least 48

hours, in an ice box maintained at about 40-45° F.

A remarkable feature of our improved soluble oil is the fact that it forms an immediate permanent emulsion with extremely hard water. For instance, extensive tests were made in water having a temporary hardness of 347 parts per million, permanent hardness of 191 parts per million, and a total hardness therefore of 538 parts per million (calculated as calcium carbonate). In order to have a standard of comparison, a hard water is used for testing emulsibility. About 0.2718 grams  $2CaSO_4 \cdot H_2O$ , 0.2540 grams  $MgSO_4$ , 0.8360 grams  $CaCO_3$ , 0.6960 grams  $MgCO_3$ , 2.824 grams  $Na_2SO_4$ , and 0.12 grams  $CaCl_2$ , are mixed into four liters of distilled water and blown with carbon dioxide until a clear solution is secured. Our improved soluble oils emulsify readily and give suitable emulsions in this extremely hard water.

Another characteristic of our product is the extremely high degree of dispersion it gives when mixed with water. The drawing shows in graphical form the results obtained with such an emulsion. The differential ratio of concentration and radius is plotted against the particle size from which it is seen that most of the particles fall within the range of 30 millimicrons or smaller. This unusually small particle size we believe accounts for the great stability of this emulsion.

Hereinabove we have given a preferred formula employing 12% mahogany soap. Another preferred embodiment using a larger amount of purified mahogany soap is as follows:

|                                                                     | Per cent |
|---------------------------------------------------------------------|----------|
| Purified mahogany soap stock (50% soap)                             | 35       |
| Soda rosin soap                                                     | 2        |
| $H_2O$                                                              | 2        |
| Junior red engine oil                                               | 61       |
| (vis. 200 sec. Saybolt at 100° F., pour 35° F., color 5-6 N. P. A.) | 40       |

In making our soluble oil on a commercial scale it is sometimes convenient to employ a purified mahogany soap in admixture with about 50% of oil, and it is also convenient to apply a soda rosin soap stock containing 40% of water. Thus a preferred formula might be made with these ingredients, using—

|                                                            | Per cent |
|------------------------------------------------------------|----------|
| Purified mahogany soap mixture                             | 23.4     |
| Soda rosin soap stock, aqueous                             | 3.6      |
| Lubricating oil, such as straw oil                         | 73       |
| (80 sec. vis. at 100° F., 35° F. pour, 1-2 N. P. A. color) |          |

From the above specific examples and from the general principles hereinabove set forth it will be seen that the proportions of purified mahogany soap to water-soluble soap and/or water must be carefully regulated but can be readily determined in accordance with the principles hereinabove stated. We do not limit ourselves to any of the specific details hereinabove described except as defined by the following claims which should be construed as broadly as the prior art will permit.

We claim:

1. A soluble oil which contains no alcohol and which will readily emulsify in extremely hard water and which consists essentially of a mineral lubricating oil having a viscosity of about 80-300 seconds Saybolt at 100° F. containing in solution about 8% to 40% of purified mahogany soap, a small amount of a preferentially water-soluble soap, and about 2.5% to 0.5% of water, the amount of water being sufficiently low to prevent separa- 75

tion of the soap when the soluble oil is exposed for an extended period to an ice bath.

2. A hard water soluble oil having about the following formula:

|                                                   | Per cent       |
|---------------------------------------------------|----------------|
| 5 Purified mahogany soap (soluble in 80% alcohol) | 8-40           |
| Soda rosin soap                                   | 1-6            |
| Water                                             | 2.5-0.5        |
| 10 Lubricating oil                                | balance to 100 |

3. A hard water soluble oil having about the following formula:

|                                   | Per cent |
|-----------------------------------|----------|
| Purified mahogany soap (oil free) | 12       |
| Soda rosin soap (dry)             | 2.5 5    |
| Water                             | 1.5      |
| Mineral oil                       | 84.0     |

ELMER WADE ADAMS.

GEORGE W. FLINT.

10